

# United States Patent

Shiba et al.

[15] 3,658,547

[45] Apr. 25, 1972

[54] SILVER HALIDE PHOTOGRAPHIC  
EMULSIONS CONTAINING  
PHENOZINE-N-OXIDES  
DESENSITIZERS

[72] Inventors: Keisuke Shiba; Reiichi Ohi; Masatoshi Sugiyama; Azusa Ohhashi; Motohiko Tsubota, all of Kanagawa, Japan

[73] Assignee: Fuji Photo Film Co., Ltd., Ashigara-Kamigum, Kanagawa, Japan

[22] Filed: Mar. 6, 1970

[21] Appl. No.: 17,316

[30] Foreign Application Priority Data

Mar. 7, 1969 Japan.....44/17259

[52] U.S. Cl.....96/101

[51] Int. Cl.....G03c 1/36

[58] Field of Search.....96/101

[56]

References Cited

UNITED STATES PATENTS

|           |        |                     |          |
|-----------|--------|---------------------|----------|
| 3,403,025 | 9/1968 | Rees et al. ....    | 96/101   |
| 3,250,618 | 5/1966 | Stewart et al. .... | 96/101 X |
| 3,340,063 | 9/1967 | Kalenda.....        | 96/101 X |
| 3,237,008 | 2/1966 | Dostes et al. ....  | 96/101 X |

Primary Examiner—Norman G. Torchin

Assistant Examiner—Won H. Louie, Jr.

Attorney—Sughrue, Rothwell, Mion, Zinn & Macpeak

[57]

ABSTRACT

Photographic silver halide emulsion and photographic elements containing same, said elements containing certain phenazine desensitizing dyes. The dyes of this invention selectively desensitize the silver halide emulsion to visible light, as contrasted with X-rays.

5 Claims, No Drawings

SILVER HALIDE PHOTOGRAPHIC EMULSIONS  
CONTAINING PHENOZINE-N-OXIDES DESENSITIZERS

## BACKGROUND OF THE INVENTION

## 1. Field of the Invention

The present invention relates to a silver halide photographic emulsion having selectively reduced sensitivity to visible light and, more particularly, to a silver halide photographic emulsion of which the sensitivity to visible light has been reduced without reducing sensitivity to X-rays.

## 2. Description of the Prior Art

Usually, photographic light-sensitive elements must be developed, after image exposure, in a dark room or under safe light and the development must also be conducted, in general, under controlled conditions of temperature, time, agitation and the like. Thus, as these developing operations must be conducted in a dark room or under safe light, various attempts have been made to allow the conducting of these operations under more convenient conditions.

In ordinary silver halide photographic emulsions, the sensitivity thereof to X-rays is in direct proportion to sensitivity to visible light.

An object of the present invention is to provide a specific silver halide photographic emulsion, the sensitivity of which to visible light has been selectively reduced without reducing the sensitivity thereof to X-rays, whereby it becomes possible to handle the light-sensitive element made from such a light-sensitive photographic emulsion under visible light after the light-sensitive element is exposed to X-rays.

Another object of the present invention is to provide a desensitizing agent capable of reducing selectively the sensitivity of a silver halide photographic emulsion to visible light without reducing the sensitivity thereof to X-rays.

Still another object of the present invention is to provide a silver halide photographic X-ray-sensitive element having a silver halide emulsion layer containing the desensitizing dye as mentioned above.

In this respect, by using an ordinary desensitizing dye, such as pinakryptol yellow, phenosafranine, methylene blue and the like, the sensitivity of a silver halide photographic emulsion to X-rays may be reduced considerably, but these materials tend to remain after development as stains.

## SUMMARY OF THE INVENTION

The inventors have found that the above objects of the present invention can be attained by incorporating into a silver halide photographic emulsion a compound represented by the general formula



or



wherein R<sub>1</sub>, R<sub>2</sub>, R<sub>3</sub>, and R<sub>4</sub> each represents a hydrogen atom, an alkyl group (e.g. lower alkyl), an aryl group (e.g. phenyl), a nitro group, a hydroxyl group, an alkoxy group (e.g. lower alkoxyl), a halogen atom, an amino group or a substituted amino group, or said R<sub>1</sub> and R<sub>3</sub> or said R<sub>2</sub> and R<sub>4</sub> may be condensed with each other to form a benzene ring.

## DETAILED DESCRIPTION OF THE INVENTION

Examples of alkyl substituting groups of the phenazine oxide derivatives represented by the above mentioned general formula are lower alkyl groups, such as methyl, ethyl, butyl and the like. Examples of halogen atoms are chlorine, bromine and the like and examples of substituted amino groups are lower alkyl-substituted amino groups, such as alkyl amino, di-alkyl amino, and acylamido group, and the like.

The use of phenazine derivatives as desensitizing dyes is known but it has never been known that the phenazine oxide derivatives employed in the present invention selectively desensitize a silver halide photographic emulsion to visible light while having much less effect upon the sensitivity of the emulsion to X-rays.

Moreover, the aforesaid compound to be used in the present invention has the advantage that when the compound is incorporated into a silver halide photographic emulsion layer of a photographic light-sensitive element, less stain is left after the light-sensitive element is developed and, further, since the absorption wave length of the compound is in the short wave length region, any stain which may remain after development, is inconspicuous.

The aforesaid phenazine oxide derivative used in the present invention may be incorporated into a silver halide photographic emulsion as a solution in a water-miscible organic solvent such as methanol, ethanol, acetone, pyridine and the like. The amount of the compound to be incorporated in the silver halide photographic emulsion is preferably  $1.5 \times 10^{-4}$  to  $1 \times 10^{-2}$  mole per mole of silver halide in the silver halide emulsion. As the silver halide photographic emulsion, there may be profitably used a silver iodobromide emulsion, a silver bromide emulsion, and a silver chloroiodo-bromide emulsion.

The silver halide photographic emulsion containing the above-mentioned desensitizing dye may be applied to any suitable support, such as a cellulose triacetate film, a polyethylene terephthalate film, a baryta-coated paper, a resin-coated paper or other plastic film.

Typical examples of the aforesaid compounds represented by the above-mentioned general formula are shown below. It should, however, be understood that the invention shall not be limited to only these compounds. The temperatures shown with the compounds are the melting or decomposition points of the corresponding compounds;

|    | Compound          | Structure | ° C.    |
|----|-------------------|-----------|---------|
| 50 | Compound (a)----- |           | 222     |
| 55 | Compound (b)----- |           | 258     |
| 60 | Compound (c)----- |           | 154-155 |
| 65 | Compound (d)----- |           | 203     |
| 70 |                   |           |         |
| 75 |                   |           |         |



50 The aforesaid phenazine oxide derivatives used in the present invention may be prepared by either of the following well known methods:

1. A Wohl-Aue reaction, wherein an aniline or naphthylamine is reacted with a nitrobenzene in a non-polar solvent, such as benzene or toluene, using potassium hydroxide as the condensing agent.
  2. A method wherein a phenazine obtained by the condensation reaction of an o-quinone and o-phenylenediamine is oxidized using hydrogen peroxide.
- 60 The invention will be further illustrated by the following example.

#### EXAMPLE

- 65 One kilogram of a gelatino silver iodobromide emulsion (containing 1 mole% iodine) was melted at 40° C. in a beaker. A desired amount of a methanol solution of the compound of this invention in a desired concentration was added to the system followed by stirring. The resultant silver halide emulsion was applied to a cellulose triacetate film in a thickness of 7.5 microns  $\pm$  0.5 micron and dried to provide a silver halide photographic light-sensitive film.
- 70 The photographic light-sensitive film thus prepared was cut into two portions. One specimen was exposed to X-rays using an X-ray source of 75 k. V. and 6 amp. through an aluminum

wedge of a definite thickness. The other specimen was exposed for 8 minutes to a daylight source through a yellow filter for safe light (More Light; made by Eastman Kodak Co.) under definite conditions.

The specimen films thus exposed were developed for 4-5 minutes at 20° C. in a developer having the following composition and then fixed;

|                               |          |
|-------------------------------|----------|
| Metol                         | 4 g.     |
| Anhydrous sodium sulfite      | 60 g. 10 |
| Hydroquinone                  | 10 g.    |
| Sodium carbonate mono-hydrate | 53 g.    |
| Potassium bromide             | 2.5 g.   |
| Water to make                 | 1 liter. |

The relative sensitivity to X-rays and the density of fog by 15 yellow light of the various specimens were measured, the results of which measurements are shown in the following table.

| No. | Compound and conc. of the solution of the compound | Amount of solution (ml.) | Relative sensitivity to X-rays | Fog density by yellow light |
|-----|----------------------------------------------------|--------------------------|--------------------------------|-----------------------------|
| 1   | None                                               | 20                       | 325                            | 3.20                        |
| 2   | Compound (a), $1 \times 10^{-3}$ mole              | 20                       | 360                            | 2.70                        |
| 3   | do                                                 | 40                       | 200                            | 0.40                        |
| 4   | do                                                 | 80                       | 100                            | 0.30                        |
| 5   | Compound (c), $1 \times 10^{-2}$ mole              | 20                       | 480                            | 0.57                        |
| 6   | do                                                 | 40                       | 430                            | 0.32                        |
| 7   | do                                                 | 80                       | 150                            | 0.20                        |
| 8   | Compound (d), $1 \times 10^{-3}$ mole              | 80                       | 325                            | 0.25                        |
| 9   | do                                                 | 200                      | 250                            | 0.20                        |
| 10  | do                                                 | 400                      | 145                            | 0.10                        |
| 11  | Compound (f), $1 \times 10^{-2}$ mole              | 20                       | 360                            | 0.52                        |
| 12  | do                                                 | 40                       | 350                            | 0.22                        |
| 13  | do                                                 | 80                       | 200                            | 0.10                        |
| 14  | Compound (h), $1 \times 10^{-2}$ mole              | 80                       | 200                            | 0.30                        |
| 15  | do                                                 | 200                      | 200                            | 0.12                        |
| 16  | do                                                 | 400                      | 200                            | 0.10                        |

What is claimed is:

1. A silver halide photographic emulsion having a reduced sensitivity to visible light and a high sensitivity to x-rays consisting essentially of a desensitizing amount of a compound represented by the general formula selected from the group consisting of



40



and



55



wherein R<sub>1</sub>, R<sub>2</sub>, R<sub>3</sub>, and R<sub>4</sub> each is selected from the group consisting of hydrogen, alkyl, aryl, nitro, hydroxyl, alkoxy, halo, amino and substituted amino, and wherein said R<sub>1</sub> and R<sub>3</sub> and said R<sub>2</sub> and R<sub>4</sub> together may be condensed with each other to form a benzene ring.

2. The silver halide photographic emulsion of claim 1 wherein said compound is incorporated into the silver halide emulsion in an amount of from  $1.5 \times 10^{-4}$  to  $1 \times 10^{-2}$  mole per mole of silver halide in said emulsion.

3. A silver halide photographic light-sensitive element for 70 X-ray photography comprising a support having thereon a layer of silver halide photographic emulsion as set forth in claim 1.

4. The silver halide photographic emulsion of claim 1, wherein said compound is a member selected from the group 75 consisting of



75





and

5

5. A silver halide photographic emulsion having a reduced sensitivity to visible light and a high sensitivity to X-rays consisting essentially of a compound selected from the group consisting of





5

10



15



20



25



30



35



40



50



said compound being incorporated into the silver halide emulsion in an amount of from  $1.5 \times 10^{-4}$  to  $1 \times 10^{-2}$  mol per mol of silver halide in said emulsion.

\* \* \* \* \*

55

60

65

70

75